

March 30, 1971

F. H. COCKS  
METHOD OF IMPROVING STRESS CORROSION RESISTANCE OF  
ALUMINUM ALLOYS  
Filed Nov. 21, 1968

3,573,117



FIG. 1.



FIG. 2.

FRANKLIN H. COCKS  
INVENTOR.

BY

*Nicholas A. Pandisso*

ATTORNEY.

1

3,573,117  
**METHOD OF IMPROVING STRESS CORROSION  
RESISTANCE OF ALUMINUM ALLOYS**  
Franklin H. Cocks, Waltham, Mass., assignor to Tyco  
Laboratories Inc., Waltham, Mass.  
Filed Nov. 21, 1968, Ser. No. 777,745  
Int. Cl. C21d 1/50; C22f 1/04

U.S. Cl. 148—159

7 Claims

## ABSTRACT OF THE DISCLOSURE

Method of heat treating aluminum base alloys of the zinc-magnesium copper series to attain improved resistance to stress corrosion. The method comprises quenching the alloy following solution treatment in liquid held at a temperature of between about 230° F. and about 260° F. followed by a two step aging treatment the first of which is conducted at a temperature between about 230° F. and about 260° F. for a period of between about 20 hours and 30 hours and the second aging step is conducted between about 310° F. and 340° F.

The invention described herein was made in the performance of work under a NASA contract and is subject to the provisions of Section 305 of the National Aeronautics and Space Act of 1958, Public Law 85-568 (72 Stat. 435; 42 U.S.C. 2457).

This invention relates to heat treatable, high strength aluminum-base alloys of the 7000 series, and more particularly to a process for heat treating such alloys to substantially increase the time to failure when exposed to corrosive environments under conditions of high stress.

Although several theories have been advanced to explain the phenomenon of stress-corrosion cracking in aluminum alloys (i.e., failure caused by the simultaneous presence of stress and a corrosive environment), perhaps the most widely accepted theory correlates cracking with the simultaneous presence of stress and localized impoverished areas at grain boundaries. These impoverished areas are believed to be anodic in nature and are formed along the grain boundaries as a result of the diffusion of certain elements out of the lattice of the solid solution to form precipitate particles at these boundaries. When the alloy is exposed to a corroding medium, galvanic action occurs and results in the development of small cracks. It is further theorized that high local stresses accelerate oxide rupture and slip step emergence and thus accelerate the galvanic action. Continued corrosion of the anodic material increases the sizes of the initial cracks which, in turn, become sharpened by further concentration of the stresses. Failure of the alloy is typically sudden and dramatic.

For structural applications, such as may be found in the aircraft industry (e.g., wing and fuselage struts) where high resistance to corrosion is also necessary, weight penalties incurred by the necessity of increasing the size of the section to safely carry the required loads can be very significant. Hence, any process which will have the effect of decreasing the susceptibility of the alloy to stress corrosion cracking, without an accompanying loss of mechanical properties, has great application.

Accordingly, the primary object of the present invention is to improve the stress corrosion resistance of aluminum-base alloys while also retaining the mechanical properties at a high level.

Another object is to provide a method of heat-treating aluminum base alloys of the copper-magnesium-zinc series which is effective in markedly improving their resistance to stress-corrosion cracking.

2

A further object is to provide a method of heat-treating selected aluminum base alloys which can be applied in whole or in part to already fabricated members and which results in improved stress corrosion resistance.

5 A more specific object is to provide a process for increasing the capability of 700 series aluminum-base alloys (e.g., aluminum alloys of the zinc-magnesium-copper series) to withstand the effects of corrosion under conditions of stress, while maintaining the strength properties of such alloys at a level of at least 95% of the high strength properties characteristic of the T6 or T651 temper. Related thereto is the additional object of providing an aluminum-base alloy of the copper-magnesium-zinc series which, when treated according to the process 10 15 of the present invention, exhibits high resistance to failure under stress-corrosion conditions and retains at least 95% of the strength properties typical of such alloys in the T6 or T651 condition.

Described briefly, the present invention comprises subjecting the alloy to a solution heat-treatment, then to an oil quench, and thereafter to a two-phase aging treatment. The first phase of the aging treatment develops near full strength in the alloy; the second phase involves overaging and develops maximum resistance to failure under 20 25 conditions of high stress and corrosion. The first phase involves more time but a lower temperature than the second phase.

Other objects and many of the attendant advantages of the present invention are described or rendered obvious 30 by the following detailed description which is to be considered together with the accompanying drawings wherein:

FIG. 1 is a plot showing typical yield strength properties versus overaging time for 7075 aluminum alloys treated according to the present invention, and

35 FIG. 2 is a plot showing with respect to overaging time the resistance to failure of 7075 aluminum alloy treated according to the present invention while subject to stress and a corrosive environment.

40 The aluminum-base alloys to which the present invention is applicable are those of the so-called 7000 series, which contain zinc as their principal alloying element but which may contain other alloying elements (e.g. copper and magnesium) as well. In particular, it is applicable to aluminum base alloys of the type containing copper in the range from about 1.2 to 2.0 weight percent, magnesium in the range from about 2.1 to 2.9 weight percent, zinc in the range from about 5.1 to 6.5 weight percent, and chromium in the range of 0.18 to 0.40 weight percent.

45 An alloy with such a composition is commonly referred to as 7075 aluminum alloy, according to the numerical designation adopted by the aluminum industry. As applied to these alloys, the invention results in greatly increased resistance to failure under conditions of stress and corrosion and the retention of at least 95% of the mechanical strength which they possess after the standard heat treatments known in the industry as the T6 and T651 temper treatments. The standard T6 temper heat treatment used in the aluminum industry for 7000 series alloys such as the

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410

TABLE I

| Alloy and temper | Ultimate strength, p.s.i. | Yield strength, 0.2% offset, p.s.i. | Elongation in two inches, percent |
|------------------|---------------------------|-------------------------------------|-----------------------------------|
| 7075-T6-----     | 73,000                    | 62,000                              | 8                                 |
| 7075-T651-----   | 76,000                    | 68,000                              | 5                                 |

Although the T6 and T651 temper treatments develop mechanical strength, it is also known that each of these treatments has the effect of rendering the alloy susceptible to catastrophic failure when exposed to corrosive environments under stress.

For example, it has been found that short transverse tensile samples of aluminum alloy 7075 which have been heat-treated in the conventional manner to T651 temper tend to fail in about 30 minutes when loaded to 65,600 p.s.i. (approximately 90% of the yield strength of specimen) in 1 M NaCl solution buffered to a pH of 4.7 and corroded with an anodic current of 0.3 ma./cm.<sup>2</sup>. Attempted improvements in the stress-corrosion resistance of the alloy have included methods in which the alloy is aged at a higher-than-normal temperature, or overaged, or age hardened at a high temperature and overaged at lower temperature. In each instance, the result has seemingly improved the resistance of the alloy to stress corrosion, but to the extent this has been achieved there has been an accompanying and significant decrease in 0.2% yield strength. For example, when 7075 alloy is overaged to the -T73 temper from the T6 temper, the 0.2% offset yield strength is reduced by about 9,000 p.s.i. This problem is overcome by the present invention.

Essentially the present invention involves solution heat treating specimens of the alloy to a temperature within the range of about 860° F. to 920° F., preferably about 900° F., for a period sufficient to allow the alloying constituents to enter into solid solution. This period ranges from a few minutes to several hours, depending on the chemical composition and thickness of the specimens. Specifically, I have found that a soaking period of approximately 60-minute duration contributes favorably to the development of optimum properties. At the conclusion of the solution heat treating phase of the process, the specimens are then quenched at a rapid rate to a temperature of about 230-260° F., preferably by immersion in an oil bath which is heated and maintained at this temperature range, preferably at about 250° F. Following quenching, the specimens are artificially aged to develop full mechanical properties, this latter treatment comprising maintaining the specimens at a temperature within the range of 230° F. to 260° F., preferably 250° F., for a period of 20-30 hours, preferably about 24 hours. This aging treatment may be accomplished by continued immersion of the articles in the quench medium, e.g., oil bath, providing the temperature of the quench medium can be maintained substantially constant. However, the quenched specimens can also be aged in an oven. At the conclusion of this aging step, the specimens are subjected to overaging by heating them to a temperature between 310° F. and 340° F., preferably about 325° F., for a period of not less than 7 and no more than about 20 hours. Preferably, to preserve optimum strength properties and to provide a high degree of resistance to stress-corrosion conditions, the articles are not cooled subsequent to the quenching and before age hardening and are overaged at about 325° F. for a period of at least 8 but not more than 18 hours, and more preferably about 12 hours.

The effect on mechanical strength and resistance to stress corrosion resulting from the process of the present invention is illustrated by the following example.

#### EXAMPLE

Eight identical specimens of 7075-T651 Alloy were prepared. These specimens were made in the conventional shape employed for strength tests, having two enlarged

end sections with a 1/4 inch O.D. and an intermediate section with an 1/8 inch O.D. and a length of 9/16 inch. The overall length of each sample was 1 1/8 inches. All of these specimens were solution heated to a temperature of 900° F. for a period of one hour. Thereafter, the specimens were immediately quenched in an oil bath maintained at a temperature of approximately 250° F. The quenched specimens were not removed from the oil bath which was maintained at a temperature of 250° F. The specimens were maintained at this temperature in the bath for a period of 24 hours to effect artificial aging. Two specimens (assigned numbers 1 and 2) were set aside for testing with no additional heat treatment. Thereafter, six specimens were placed in another oil bath which was maintained at a temperature of 325° F. Two specimens (assigned numbers 3 and 4) were removed after four hours of overaging. Two other specimens (numbered 5 and 6) were removed from the bath after seven hours and forty-five minutes of overaging. The final two specimens (numbered 7 and 8) were removed from the bath after eighteen hours. Specimens 1, 3, 5 and 7 were subjected to yield strength tests. Specimens 2, 4, 6 and 8 were subjected to corrosion resistance tests. The yield strength tests were conducted in accordance with established procedures for 0.2 percent offset yield stress tests. The corrosion resistance tests consisted of loading the specimens to 90% of their respective 0.2 percent offset yield strengths in a 1 M NaCl solution buffered to a pH of 4.7 and corroded with an anodic current of 0.3 ma./cm.<sup>2</sup>. The solution was circulated at a rate of 220 ml./min. and was maintained at a temperature of 30° C.

Table II illustrates the results of the yield strength and corrosion resistance tests.

TABLE II

|           | Yield strength, 0.2% offset (p.s.i.) | Corrosion resistance time to failure (min.) |
|-----------|--------------------------------------|---------------------------------------------|
| Specimen: |                                      |                                             |
| 1-----    | 74,200                               | 14                                          |
| 2-----    | 74,700                               | 5.5                                         |
| 3-----    | 73,800                               | 420                                         |
| 4-----    | 70,900                               | 6,000                                       |
| 5-----    |                                      |                                             |
| 6-----    |                                      |                                             |
| 7-----    |                                      |                                             |
| 8-----    |                                      |                                             |

It is believed obvious that specimens 6 and 8 have corrosion resistances many times greater than those of specimens 2 and 4. Comparison of the corrosion resistances of these specimens with the corresponding characteristic of conventional 7075-T651 alloy indicates that the process of the present invention is capable of yielding more than a 100 fold increase in stress corrosion resistance with only a minor, as low as 1%, decrease in yield strength.

A number of other tests conducted on specimens heat treated as above described but with the overaging treatment varied as to time, demonstrate that the overaging treatment initially has little effect on yield strength and seemingly produces a slight gain in strength. In this connection reference is had to FIG. 1 which is a plot of typical yield strength as a function of overaging time where the overaging is conducted at a temperature of 325° F. It is believed apparent that after approximately six hours of overaging treatment, the yield strength begins to decrease as a function of overaging time. Significantly, this tendency toward a decrease in yield strength marks the beginning of a drastic improvement in the time to failure of the specimens when subjected to the stress corrosion tests. This is demonstrated by FIG. 2 which illustrates how the stress corrosion resistance, taken as the time to failure under the application of the stress load, varies with overaging time where the overaging is conducted at a temperature of 325° F.

As indicated by FIG. 2, it is to be noted that specimens artificially aged as above described, but not subjected to overaging treatment, will fail within an average of about 12 to 14 minutes. FIG. 2 clearly shows that there is no substantial increase in stress corrosion resistance if the alloy is overaged for about six hours or less. However, if the alloy is overaged for more than about six hours, the resistance to stress corrosion will improve markedly. The overaging treatment initially has little degrading effect and, as indicated by the yield strength curve of FIG. 1, seemingly even produces a slight gain in the alloy's tensile strength properties. However, after approximately six hours of overaging at 325° F., the yield strength begins to decrease as a function of overaging time.

Considering the plots of FIGS. 1 and 2 together, it is believed apparent that overaging for a period between approximately 7 hours to approximately no more than 18 hours is necessary in order to achieve an optimum combination of stress corrosion resistance and yield strength. It is significant that if the specimens are overaged at 325° F. for a period of 18 hours, the yield strength decreases from approximately 73,000 p.s.i. which is characteristic of the conventional T651 temper to approximately 71,000 p.s.i., a loss of only about 2.7%. On the other hand, the stress corrosion resistance increases by a factor of more than 100.

The significant improvement in stress corrosion resistance which is achieved is due to the unique combination of steps which make up the process of the invention. It has been determined that if the solutionized alloy is not quenched to a temperature in the neighborhood of 230-260° F., the stress corrosion resistance and strength of the alloy will be no greater than that achieved with the conventional T73 temper treatment. Quenching in water at room temperature (as in the T6, T651 and T73 temper treatments), or even in warm water maintained at a temperature of 150° F. as mentioned in U.S. Pat. 3,231,435, will not provide the same results as quenching at the higher temperature utilized in the present invention. Furthermore, the use of an oil quench provides more uniform cooling and hence minimizes development of internal stresses. Quenching in oil heated to 250° F. provides a more homogeneous and less irregular heat transfer from the alloy specimens than does water quenching. As a result, the subsequent distribution of the precipitate particles which are formed after age hardening and overaging gives an improved combination of strength and resistance to stress corrosion. Furthermore, the alloy is more nearly free of internal stresses which unfavorably affect its stability. Deviation by as much as 10-15 degrees from the range of 230-260° F. for the quench bath temperature is permissible and, depending on the composition and size of the alloy specimens, will not appreciably effect the strength properties of the heat treated alloy. Aging the alloy at a temperature appreciably lower than 230° F. will have the tendency of slowing up the aging process, with the result that maximum stress-corrosion resistance will not be attained as easily by the overaging treatment. Aging the alloy at a temperature appreciably above 260° F. tends to adversely affect the beneficial effect of the subsequent overaging treatment since the distribution of precipitates caused by the age hardening treatment tends to be excessively coarsened. The same coarsening tends to occur if overaging itself is conducted at a temperature appreciably above 340° F.

Although the example set forth above is concerned with 7075 originally in the T651 temper, the same improvement in stress corrosion resistance occurs if the alloy is originally in the T6 temper or any other heat-treated state. Similarly the invention is applicable to other aluminum alloys of the 7000 series as, for example, the 7001 alloy which characteristically includes 2.6 to 3.4 percent magnesium, 6.8 to 8.0 percent zinc, 1.6 to 2.6 percent copper, and 0.18 to 0.40 chromium. For the

latter alloy and other alloys of the 7000 series, the temperature of the quench bath and the optimum temperatures and times for the aging and overaging phases may be somewhat greater or less according to the specific composition of the alloy. However, the solutionizing temperature is essentially as herein prescribed. Except for these differences in operation conditions, the process is essentially the same, yielding a substantially material increase in stress corrosion resistance at the expense of only a slight decrease in yield strength. Other tensile properties, such as ultimate tensile strength and the percentage elongation over a given length, e.g., two inches of specimen, are modified to substantially the same extent as yield strength by this process. Hence on balance, aluminum alloys of the 7000 series are materially improved and their usefulness for structural applications is greatly enhanced by this invention.

A further important advantage of the invention is that it is applicable even after the alloy has been shaped, e.g., by rolling, into structural parts. Still another advantage is that it may be practiced successfully without conforming strictly to the specific procedure set forth above. Thus the specimens may be allowed to cool to room temperature after being quenched and before being subjected to artificial aging. It is also permissible to allow the alloy to cool to a temperature lower than the aging temperature before subjecting it to the overaging treatment. With any or all of these variations in procedure, the heat treated specimens will exhibit substantially the same mechanical properties and the same stress corrosion resistance as is achieved with the preferred procedure described above.

It is appreciated that other variations and modifications of the invention that do not depart from the principles herein set forth will be obvious to persons skilled in the art. Accordingly, it is to be understood that the matter contained in the foregoing description and shown in the accompanying drawings is to be interpreted in an illustrative rather than limiting sense and that the scope of the invention is to be determined solely from the appended claims construed in the light of this specification.

What is claimed is:

1. A process for heat treating a high-strength aluminum base alloy of the zinc-magnesium-copper series in which the zinc content is greater than each of the magnesium and copper contents to reduce its susceptibility to stress-corrosion cracking while retaining its high strength properties comprising, heating the alloy to a temperature of between about 850° F. and about 915° F. for a period of time sufficient to allow the constituents of said alloy to enter into solid solution, quenching said heated alloy, aging the quenched alloy by heating it to a temperature between about 230° F. and about 260° F. for a period of between about 20 hours and 30 hours, and thereafter heating the aged alloy to a temperature between about 310° F. and 340° F. for a period of no less than about 7 and no more than about 20 hours, said alloy being quenched from the temperature of solution heat treatment into a liquid to a temperature of between about 230° F. and about 260° F.
2. The process of claim 1 wherein said alloy is quenched in an oil bath.
3. The process of claim 1 wherein said alloy is aged at a temperature of about 250° F. for a period of about 24 hours.
4. The process of claim 1 wherein said aged alloy is heated to a temperature of about 325° F. for a period of between about 7 hours and about 18 hours.
5. The process of claim 1 wherein said alloy comprises by weight about 1.2 to 2.0% copper, about 2.1 to 2.9% magnesium, and about 5.1 to 6.5% zinc and 0.18 to 0.40% chromium.
6. The process of claim 1 wherein said alloy comprises by weight 1.6 to 2.6% copper, 2.6 to 3.4% magnesium, 6.8 to 8.0% zinc, and 0.18 to 0.40% chromium.

7. A process for heat treating articles of aluminum base alloys of the zinc-magnesium-copper series in which the zinc content is greater than each of the magnesium and copper contents so as to increase the resistance of the articles to failure when exposed to a corrosive medium while under conditions of high stress and also to develop high strength in said articles, said process comprising:

heating said articles to a temperature of between about 850° F. and about 915° F. for a period sufficient to dissolve the alloying constituents into solid solution; quenching said articles in oil heated to a temperature of between about 230° F. and about 260° F.; aging said articles in said oil at said temperature of between about 230° F. and about 260° F. for between about 20 hours and 30 hours; and

overaging said articles at a temperature of between 310° F. to 340° F. for a period of at least 7 and no more than 20 hours.

#### References Cited

##### UNITED STATES PATENTS

|           |         |                      |         |
|-----------|---------|----------------------|---------|
| 2,242,944 | 5/1941  | Dix et al. -----     | 148—159 |
| 2,695,253 | 11/1954 | Schaaber -----       | 148—159 |
| 3,171,760 | 3/1965  | Vernam et al. -----  | 148—159 |
| 3,231,435 | 1/1966  | Rotsell et al. ----- | 148—159 |

##### FOREIGN PATENTS

|         |        |                     |         |
|---------|--------|---------------------|---------|
| 544,439 | 4/1942 | Great Britain ----- | 148—159 |
|---------|--------|---------------------|---------|

15 CHARLES N. LOVELL, Primary Examiner

UNITED STATES PATENT OFFICE  
CERTIFICATE OF CORRECTION

Patent No. 3573117 Dated March 30, 1971

Inventor(s) FRANKLIN H. COCKS

It is certified that error appears in the above-identified patent and that said Letters Patent are hereby corrected as shown below:

L

Column 3, lines 6 and 7, the values "8" and "5" in Table I are changed to "5" and "8" respectively.

Signed and sealed this 22nd day of June 1971.

(SEAL)

Attest:

EDWARD M. FLETCHER, JR.  
Attesting Officer

WILLIAM E. SCHUYLER, JR.  
Commissioner of Patents

L